

1

3,379,533

**DYES DERIVED FROM 1,2 - DISUBSTITUTED - 3,5-PYRAZOLIDINEDIONES AND PHOTOGRAPHIC ELEMENTS CONTAINING SUCH DYES**

Philip W. Jenkins and Leslie G. S. Brooker, Rochester, N.Y., assignors to Eastman Kodak Company, Rochester, N.Y., a corporation of New Jersey

No Drawing. Filed June 10, 1963, Ser. No. 286,449  
7 Claims. (Cl. 96—102)

This invention is related to dyes for photography and more particularly to dyes derived from 1,2-disubstituted-3,5-pyrazolidinediones and their use as sensitizers for photographic silver halide emulsions and/or bleachable filter dyes for light absorbing layers in photographic elements.

It is known that certain cyanine dyes are useful for spectral sensitization of silver halide emulsions, that is, for extending the sensitivity of the silver halide to light of longer wavelengths.

It is also known to use certain bleachable dyes in light-filtering hydrophilic layers in light-sensitive photographic elements. Such light-filtering layers may be coated over the light-sensitive layer, between two differently sensitized light-sensitive layers, between a light-sensitive layer and the support or on the side of the support opposite to the side bearing a light-sensitive layer. Dyes useful for filter layers must not only absorb light of the desired wavelengths but must be readily bleachable and/or removable during the normal photographic processing operations. New sensitizing and/or light-filtering dyes are desired for use in photographic elements.

It is therefore an object of our invention to provide a new class of dyes derived from 1,2-disubstituted-3,5-pyrazolidinediones.

A further object is to provide new cyanine, merocyanine, styryl and holopolar dyes derived from 1,2-disubstituted-3,5-pyrazolidinediones that are valuable for use in photographic elements.

Another object is to provide a synthesis for making our new dyes.

Another object is to provide photographic silver halide emulsions containing our new dyes.

Still another object is to provide photographic elements comprising a support, at least one hydrophilic colloid layer containing light-sensitive silver halide and at least one hydrophilic layer containing at least one of our dyes.

Still other objects will become apparent from a consideration of the following specification and claims.

These and other objects of our invention are accomplished by synthesizing and using the dyes of our invention which are derived from a compound having the formula:



Wherein R and R' each represents the same or a different group selected from the class consisting of alkyl groups, e.g., methyl, ethyl, phenethyl, propyl, butyl, hexyl, cyclohexyl, dodecyl, octadecyl, etc. and aryl groups, e.g., phenyl, 4-methylphenyl, 4-methoxyphenyl, etc.

2

The dyes of our invention include those represented by the formulas:

II



10 III



V



and

V



wherein R and R' are as defined previously; R<sup>2</sup> represents an alkyl group, e.g., methyl, carbethoxymethyl, ethyl, carbethoxyethyl, carboxyethyl, propyl, butyl, 4-sulfonybutyl, hexyl, dodecyl, octadecyl, etc.; or an aryl group, e.g., phenyl, 4-methylphenyl, etc.; L and L' each represents a methine or a substituted methine group (e.g., —CH= or —CR<sup>5</sup>= where R<sup>5</sup> represents an alkyl group, such as methyl, ethyl, butyl, hexyl, decyl, etc.; or an aryl group, such as phenyl, tolyl, etc.); n represents an integer of from 1 to 4; r represents an integer of from 1 to 3; Z represents the nonmetallic atoms required to complete a 5 to 6 membered heterocyclic nucleus selected from the class of nuclei consisting of those of the thiazole series (e.g., thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, etc.), those of the benzothiazole series (e.g., benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole, etc.), those of the naphthothiazole series (e.g.,  $\alpha$ -naphthothiazole,  $\beta$ -naphthothiazole, 5-methoxy- $\beta$ -naphthothiazole, 5-ethoxy- $\beta$ -naphthothiazole, 8-methoxy- $\alpha$ -naphthothiazole, 7-methoxy- $\alpha$ -naphthothiazole, etc.), those of the thionaphtheno-7',6',4,5-thiazole series (e.g., 4'-methoxythianaphtheno-7',6',4,5-thiazole, etc.), those of the

oxazole series (e.g., 4-methyloxazole, 5-methyloxazole, 4-phenyloxazole, 4,5-diphenyloxazole, 4-ethyloxazole, 4,5-dimethyloxazole, 5-phenyloxazole, etc.), those of the benzoxazole series (e.g., benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole, etc.), those of the naphthoxazole series (e.g.,  $\alpha$ -naphthoxazole,  $\beta$ -naphthoxazole, etc.), those of the selenazole series (e.g., 4-methylselenazole, 4-phenylselenazole, etc.), those of the benzoselenazole series (e.g., benzoselenazole, 5-chlorobenzoselenazole, 5-methoxybenzoselenazole, 5-hydroxybenzoselenazole, tetrahydrobenzoselenazole, etc.), those of the naphthoselenazole series (e.g.,  $\alpha$ -naphthoselenazole,  $\beta$ -naphthoselenazole, etc.), those of the thiazoline series (e.g., thiazoline, 4-methylthiazoline, etc.), those of the 2-quinoline series (e.g., quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the 4-quinoline series (e.g., quinoline, 6-methoxyquinoline, 7-methylquinoline, 8-methylquinoline, etc.), those of the 1-isoquinoline series (e.g., 1-isoquinoline, 3,4-dihydro-1-isoquinoline, etc.), those of the 3-isoquinoline series (e.g., 3-isoquinoline, 6-methyl-3-isoquinoline, etc.), those of the 3,3-dialkylindolenine series (e.g., 3,3-dimethylindolenine, 3,3,5-trimethylindolenine, 3,3,7-trimethylindolenine, etc.), the pyridine series (e.g., 2-pyridine, 4-pyridine, 5-methyl-2-pyridine, etc.), those of the imidazole series (e.g., imidazole, 1-ethyl-4-phenylimidazole, 4,5-dimethylimidazole, etc.), those of the benzimidazole series (e.g., benzimidazole, 1-butyl-4-methylbenzimidazole, 1-ethyl-4-phenylbenzimidazole, 4,5-dichlorobenzimidazole, etc.), and those of the naphthimidazole series (e.g., 1-methyl- $\alpha$ -naphthimidazole,  $\beta$ -naphthimidazole, 5-methoxy- $\beta$ -naphthimidazole, etc.); W and W' each represent the nonmetallic atoms necessary to complete the same or a different 5 to 6 membered heterocyclic nucleus selected from those of the thiazole series, the benzothiazole series, the naphthothiazole series, the oxazole series, the benzoxazole series, the naphthoxazole series, the selenazole series, the benzoselenazole series, the naphthoselenazole series, the thiazoline series, the 2-quinoline series, the 4-quinoline series, the 1-isoquinoline series, the 3-isoquinoline series, the 3,3-dialkylindolenine series, and the pyridine series all as described with illustrative examples for Z, however, W and W' do not include the nuclei of the imidazole series, the benzimidazole series or the naphthimidazole series; R<sup>3</sup> and R<sup>4</sup> each represents the same or a different alkyl group, e.g., methyl, ethyl, 2-cyanomethyl, propyl, butyl, hexyl, octadecyl, etc.; and m represents an integer of from 1 to 2; and p and q each represent an integer from 1 to 2.

Our dyes are valuable for use in photographic elements. Certain of the dyes have sensitizing properties for silver halide emulsions while others are easily bleachable by photographic processing solutions and can therefore be used in the preparation of bleachable filter or antihalation layers. Some of our dyes are useful in filter layers coated over the light-sensitive layer(s) or between two or more light-sensitive layers which may be differently sensitized as in elements for color photography.

In general the dyes of our invention are produced to advantage by heating the 1,2-disubstituted-3,5-pyrazolidinedione or its 4-substituted derivative with the appropriate intermediate in a suitable inert solvent, preferably in the presence of a basic condensing agent. The condensation reactions are carried out to advantage by heating the reaction mixture to a temperature between room temperature and the reflux temperature. These conditions are used in the following general syntheses.

Any of the well known basic condensing agents are used, such as the trialkylamines, e.g., triethylamine, tri-n-

propylamine, triisopropylamine, tri-n-butylamine, etc., the N,N-dialkylanilines, e.g., N,N-dimethylaniline, N,N-diethylaniline, etc., the N-alkylpiperidines, e.g., N-methylpiperidine, N-ethylpiperidine, etc.

Inert solvents used to advantage include methanol, ethanol, propanol, cyclohexane, pyridine, acetic anhydride, etc.

The merocyanine dyes of Formula II are produced by condensing (as indicated above) the appropriate compound of Formula I with an intermediate represented to advantage with the formula:



wherein R, p and Z are as described previously, Y represents a group, such as ethyl (to produce a simple merocyanine),  $\beta$ -acetanilidovinyl or thioacetylylidene (to produce a merocarbocyanine), or 4-methoxybutadienyl, or 4-anilinovinyl-1,3-butadienyl (to produce a merodicarbocyanine dye), and X<sup>⊖</sup> represents any acid anion, e.g., chloride, bromide, methylsulfate, ethylsulfate, p-toluenesulfonate, perchlorate, etc. The Y group can also be methyl when 4-(5-acetanilido-2,4-pentadienylidene)-1,2-substituted-3,5-pyrazolidinedione is used in the condensation reaction.

The oxonols of Formula III are prepared to advantage by condensing the appropriate compound of Formula I with diethoxymethyl acetate (to give a monomethinoxonol), trimethoxypropene (to give a trimethinoxonol) and 1-anilino-5-phenylimino-1,3-pentadiene hydrochloride (to give a pentamethinoxonol).

The holopolar dyes of Formula IV are prepared to advantage by condensing the appropriate compound of Formula I with a compound represented by the formula:



wherein R<sup>2</sup>, p, q, W, W' and X<sup>⊖</sup> are as defined previously and R<sup>6</sup> represents an alkyl group or an aryl group.

The styryl dyes of Formula V are prepared to advantage by condensing a compound of Formula I with an intermediate such as p-dimethylaminobenzaldehyde or p-dimethylaminocinnamaldehyde. No basic condensing agent is needed for these reactions.

The intermediates of Formulas VI, VII and the others used (to condense with our new intermediate of Formula I) are known in the art and need not be described further.

The following representative dyes and their syntheses will serve to illustrate but not limit our invention.

Dye 1.—4-(3-ethyl-2-benzothiazolinylidene)-1,2-diphenyl-3,5-pyrazolidinedione



65

1,2-diphenyl-3,5-pyrazolidinedione (1 mol., 2.5 g.), 3-ethyl-2-ethylthiobenzothiazolium ethylsulfate (1 mol., 3.6 g.), and triethylamine (1 mol., 1.0 g.) were dissolved in ethanol (25 ml.), and the solution was heated under reflux for fifteen minutes. The mixture was chilled overnight, and the crude product was isolated by filtration, washed with methanol, and dried. After two recrystallizations from pyridine and methanol, the yield of pure dye was 1.95 g. (47%), M.P. 249.0–250.5° C.

5

Dye 2.—4-(1-ethyl-2-naphtho[1,2-d]thiazolinylidene)-1,2-diphenyl-3,5-pyrazolidinedione



1,2-diphenyl-3,5-pyrazolidinedione (1 mol., 2.5 g.), 1-ethyl-2-ethylthionaphtho[1,2-d]thiazolium ethylsulfate (1 mol., 4.1 g.), and triethylamine (1 mol., 1.0 g.) were dissolved in ethanol (35 ml.), and the solution was heated under reflux for fifteen minutes. The mixture was chilled overnight, and the crude product was isolated by filtration, washed with methanol, and dried. After two recrystallizations from pyridine and methanol, the yield of pure dye was 3.2 g. (69%), M.P. 251.0–253.0° C.

Dye 3.—4-[1-(3,3-trimethyl-2-indolinylidene)ethylidene]-1,2-diphenyl-3,5-pyrazolidinedione



1,2-diphenyl-3,5-pyrazolidinedione (1 mol., 1.25 g.), 2- $\beta$ -acetanilidovinyl-1,3,3-trimethyl-3H-indolium iodide (1 mol., 2.25 g.), and triethylamine (1 mol., 0.5 g.) were dissolved in ethanol (20 ml.), and the solution was heated under reflux for twenty-five minutes. The mixture was chilled overnight, and the crude product was isolated by filtration, washed with methanol, and dried. After two recrystallizations from pyridine and methanol, the yield of pure dye was 1.4 g. (64%), M.P. 272.5–274.0° C. dec.

Dye 4.—4-[3-ethyl-2-benzoxazolinylidene]ethylidene]-1,2-dimethyl-3,5-pyrazolidinedione



1,2-dimethyl-3,5-pyrazolidinedione (1 mol., 0.45 g.), 2- $\beta$ -acetanilidovinyl-3-ethylbenzoxazolium iodide (1 mol., 1.45 g.), and triethylamine (1 mol., 0.35 g.) were dissolved in ethanol (10 ml.), and the solution was heated under reflux for twenty minutes. The mixture was chilled overnight, and the first crop of crude product was isolated by filtration, washed with methanol, and dried. The mother liquor and washes were combined and concentrated to dryness under reduced pressure. The residue was taken up in methanol (10 ml.), and the solution was diluted with water (100 ml.). After chilling, the second crop of product was isolated by filtration and dried. The two crops of product were combined, and after two recrystallizations from methanol and water, the yield of pure dye was 0.6 g. (60%), M.P. 243.0–244.5° C. dec.

Dye 5.—4-[3-ethyl-2-benzothiazolinylidene]ethylidene]-1,2-diphenyl-3,5-pyrazolidinedione



1,2-diphenyl-3,5-pyrazolidinedione (1 mol., 1.25 g.), 2- $\beta$ -acetanilidovinyl-3-ethylbenzothiazolium iodide (1 mol.,

6

2.25 g.), and triethylamine (1 mol., 0.5 g.) were dissolved in ethanol (25 ml.), and the solution was heated under reflux for twenty minutes. The mixture was chilled overnight, and the crude product was isolated by filtration, washed with methanol, and dried. After two recrystallizations from pyridine and methanol, the yield of pure dye was 2.1 g. (95%), M.P. 259.5–260.5° C. dec.

Dye 6.—4-[3-ethyl-2-benzothiazolinylidene]isopropylidene]-1,2-diphenyl-3,5-pyrazolidinedione



3-ethyl-2-thioacetylylidenebenzothiazoline (1 mol., 2.4 g.) and methyl p-toluenesulfonate (1 mol., 1.9 g.) were mixed and heated on a steam bath for one hundred minutes. The resulting solid cake was ground to a fine powder under ether. The mixture was filtered, and the precipitate was washed with ether. This precipitate together with 1,2-diphenyl-3,5-pyrazolidinedione (1 mol., 2.5 g.) and triethylamine (1 mol., 1.0 g.) was dissolved in ethanol (25 ml.), and the solution was heated under reflux for twenty minutes. The mixture was chilled overnight, and the crude product was isolated by filtration, washed with methanol, and dried. After two recrystallizations from pyridine and methanol, the yield of pure dye was 3.7 g. (82%), M.P. 287.0–289.0° C. dec.

Dye 7.—4-[1-ethyl-2-naphtho[1,2-d]thiazolinylidene]ethylidene]-1,2-dimethyl-3,5-pyrazolidinedione



1,2-dimethyl-3,5-pyrazolidinedione (1 mol., 0.45 g.), 2- $\beta$ -anilinovinyl-1-ethylnaphtho[1,2-d]thiazolium p-toluenesulfonate (1 mol., 1.7 g.), acetic anhydride (1 mol. +100%, 0.65 g.), and triethylamine (1 mol. +100%, 1.00 g.) were dissolved in ethanol (10 ml.), and the solution was heated under reflux for twenty minutes. The mixture was chilled overnight, and the crude product was isolated by filtration, washed with methanol, and dried. After two recrystallizations for methanol, the yield of pure dye was 0.7 g. (57%), M.P. 295.5–297.0° C. dec.

Dye 8.—4-[1-ethyl-2-naphtho[1,2-d]thiazolinylidene]isopropylidene]-1,2-dimethyl-3,5-pyrazolidinedione



1-ethyl-2-thioacetylylidenebenzothiazoline (1 mol., 2.85 g.) and methyl p-toluenesulfonate (1 mol., 1.85 g.) were mixed and heated on a steam bath for forty minutes. This crude product together with 1,2-dimethyl-3,5-pyrazolidinedione (1 mol., 1.30 g.) and triethylamine (1 mol., 1.0 g.) was dissolved in ethanol (30 ml.), and the solution was heated under reflux for twenty minutes. The mixture was chilled overnight, and the crude product was isolated by filtration, washed with methanol, and dried. After two recrystallizations from pyridine and

methanol, the yield of pure dye was 2.35 g. (62%), M.P. 264.0-265.0° C. dec.

Dye 9.—4[(1-ethyl-2(1H)-quinolylidene)ethylidene]-1,2-diphenyl-3,5-pyrazolidinedione



1,2-diphenyl-3,5-pyrazolidinedione (1 mol., 2.5 g.), 2- $\beta$ -anilinovinyl-1-ethylquinolinium iodide (1 mol., 4.0 g.), acetic anhydride (1 mol.+100%, 2.0 g.), and triethylamine (1 mol., 2.0 g.) were dissolved in ethanol (25 ml.), and the solution was heated under reflux for twenty minutes. The mixture was chilled overnight, and the crude product was isolated by filtration, washed with methanol, and dried. After two recrystallizations from pyridine and methanol, the yield of pure dye was 2.05 g. (47%), M.P. 271.5-273.0° C. dec.

Dye 10.—4[(1-ethyl-4(1H)-quinolylidene)ethylidene]-1,2-diphenyl-3,5-pyrazolidinedione



1,2-diphenyl-3,5-pyrazolidinedione (1 mol., 2.5 g.), 4- $\beta$ -anilinovinyl-1-ethylquinolinium iodide (1 mol., 4.0 g.), acetic anhydride (1 mol.+100%, 2.0 g.), and triethylamine (1 mol., 2.0 g.) were dissolved in ethanol (25 ml.), and the solution was heated under reflux for twenty minutes. The mixture was chilled overnight, and the crude product was isolated by filtration, washed with methanol, and dried. After two recrystallizations from pyridine and methanol, the yield of pure dye was 2.4 g. (55%), M.P. 288.0-289.5° C. dec.

Dye 11.—4-[4-(3-ethyl-2-benzoxazolylidene)-2-butenylidene]-1,2-dimethyl-3,5-pyrazolidinedione



1,2-dimethyl-3,5-pyrazolidinedione (1 mol., 0.45 g.), 2-(4-methoxybutadienyl)-3-ethylbenzoxazolium iodide (1 mol., 1.15 g.), and triethylamine (1 mol., 0.35 g.) were dissolved in ethanol (10 ml.), and the solution was heated under reflux for twenty minutes. The reaction mixture was cooled and diluted with water (200 ml.). The dye suspension was chilled overnight, and the crude product was collected by filtration and dried. The desired dye was extracted from the crude product with boiling benzene (125 ml.). The dye was precipitated from the benzene solution by the addition of ligroin (100 ml., B.P. 100-115° C.) and, after chilling, was isolated by filtration. After one recrystallization from benzene and ligroin (B.P. 100-115° C.), the yield of pure dye was 0.2 g. (18%), M.P. 222.5-224.5° C. dec.

Dye 12.—4-[4-(3-ethyl-2-benzothiazolylidene)-2-butenylidene]-1,2-diphenyl-3,5-pyrazolidinedione



1,2-diphenyl-3,5-pyrazolidinedione (1 mol., 2.5 g.), 2-(4-anilinovinyl-1,3-butadienyl)-3-ethylbenzothiazolium iodide (1 mol., 4.35 g.), acetic anhydride (1 mol.+100%, 2.0 g.), and triethylamine (1 mol.+100%, 3.0 g.) were dissolved in ethanol (25 ml.), and the solution was heated under reflux for twenty minutes. The reaction mixture was cooled and diluted with water (150 ml.). The dye suspension was chilled overnight, and the crude product was collected by filtration. This damp product was boiled with 50 ml. of methanol. After chilling the mixture overnight, the methanol was decanted and the residual gum dissolved in pyridine. This solution was filtered and diluted with methanol. The solution was chilled, and the crude dye was isolated by filtration and dried. After two recrystallizations from pyridine and methanol, the yield of pure dye was 0.65 g. (14%), M.P. 225.5-227.5° C. dec.

Dye 13.—4-[6-(3-ethyl-2-benzoxazolylidene)-2,4-hexadienylidene]-1,2-diphenyl-3,5-pyrazolidinedione



4 - (5 - acetanilido-2,4-pentadienylidene)-1,2-diphenyl-3,5-pyrazolidinedione (1 mol., 2.25 g.), 3-ethyl-2-methylbenzoxazolium iodide (1 mol., 1.45 g.), and triethylamine (1 mol., 0.5 g.) were dissolved in methanol (15 ml.), and the solution was heated under reflux for fifteen minutes. The crude dye was isolated from the hot reaction mixture by filtration. After one recrystallization from cresol and methanol containing piperidine, the yield of pure dye was 0.17 g. (7%), M.P. 174.5-176.5° C. dec.

Dye 14.—4-[6-(3-ethyl-2-benzothiazolylidene)-2,4-hexadienylidene]-1,2-diphenyl-3,5-pyrazolidinedione



4-(5-acetanilido-2,4-pentadienylidene)-1,2-diphenyl-3,5-pyrazolidinedione (1 mol., 2.25 g.), 3-ethyl-2-methylbenzothiazolium iodide (1 mol., 1.55 g.), and triethylamine (1 mol., 0.5 g.) were dissolved in ethanol (15 ml.), and the solution was heated under reflux for ten minutes. The reaction mixture was chilled, and the crude product was isolated by filtration, washed with methanol, and dried. After one recrystallization from pyridine and methanol, the yield of pure dye was 1.4 g. (57%), M.P. 142.0-144.0° C. dec.

Dye 15.—4-[1,3-di(3-ethyl-2-benzothiazolylidene)isopropylidene]-1,2-diphenyl-3,5-pyrazolidinedione



3,3' - diethyl - 9 - phenylthiothiacarbocyanine iodide (1 mol., 12.0 g.), 1,2-diphenyl-3,5-pyrazolidinedione (1 mol.+10%, 5.5 g.), and triethylamine (1 mol., 2.0 g.) were dissolved in pyridine (50 ml.), and the solution was

heated under reflux for twenty minutes. The hot reaction mixture was cooled and diluted with ether (400 ml.). After chilling the mixture overnight, the ether was decanted, and the residue was boiled with methanol (50 ml.). The mixture was chilled, and the crude product was isolated by filtration, washed with methanol, and dried. Two recrystallizations from pyridine and methanol gave 5.6 g. (46%) of a green powder with a gold reflex, melting at 185.5-187.5° (dec. at about 283° C.). Two recrystallizations of a portion of this dye (1.0 g.) from benzene gave 0.60 g. (60% recovery) of dark red crystals melting at 301.0-303.0° C. dec.

A second portion of this dye (1.0 g.) was recrystallized twice from *m*-xylene and gave 0.45 g. (45% recovery) of dark red crystals melting at 302.0-304.0° C. dec.

Dye 16.—4-[1,3-di(1-ethyl-2-naphtho{1,2-d}thiazolinylidene)-isopropylidene]-1,2-diphenyl-3,5-pyrazolidinedione



3,3'-diethyl-9-ethylthio-4,5,4',5'-dibenzothiacarbo-cyanine ethylsulfate (1 mol., 3.25 g.), 1,2-diphenyl-3,5-pyrazolidinedione (1 mol. + 10%, 1.4 g.), and triethylamine (1 mol., 0.5 g.) were dissolved in pyridine (15 ml.), and the solution was heated under reflux for twenty minutes. The reaction mixture was cooled and diluted with ether (250 ml.). After chilling the mixture overnight, the ether was decanted and the residue was boiled with methanol (50 ml.). The mixture was chilled, and the crude product was isolated by filtration, washed with methanol, and dried. After two recrystallizations from pyridine and methanol the yield of pure dye was 1.1 g. (31%), M.P. 290.5-292.0° C. dec.

Dye 17.—4-p-dimethylaminobenzylidene-1,2-diphenyl-3,5-pyrazolidinedione



1,2-diphenyl-3,5-pyrazolidinedione (1 mol., 2.5 g.) and *p*-dimethylaminobenzaldehyde (1 mol., 1.5 g.) were dissolved in ethanol (25 ml.), and the solution was heated under reflux for twenty-five minutes. The reaction mixture was chilled overnight, and the crude product was isolated by filtration, washed with ethanol, and dried. After two recrystallizations from pyridine and methanol, the yield of pure dye was 3.2 g. (84%), M.P. 268.0-269.0° C. dec.

Dye 18.—4-p-dimethylaminocinnamylidene-1,2-diphenyl-3,5-pyrazolidinedione



1,2-diphenyl-3,5-pyrazolidinedione (1 mol., 2.5 g.) and *p*-dimethylaminocinnamaldehyde (1 mol., 1.75 g.) were dissolved in ethanol (25 ml.), and the solution was heated under reflux for twenty-five minutes. The reaction mixture was chilled overnight, and the crude product was isolated by filtration, washed with ethanol, and dried. After two recrystallizations from the pyridine and methanol, the yield of pure dye was 2.2 g. (54%), M.P. 245.0-247.0° C. dec.

5  
10

10  
Dye 19.—Bis-(1,2-diphenyl-4-pyrazolidine-3,5-dione)methineoxonol



15  
20  
25  
1,2-diphenyl-3,5-pyrazolidinedione (1 mol., 5.05 g.), diethoxymethyl acetate (1 mol. + 10%, 1.8 g.), and triethylamine (1 mol., 2.0 g.) were dissolved in ethanol (25 ml.), and the solution was heated under reflux for fifteen minutes. The reaction mixture was cooled and diluted with glacial acetic acid (5 ml.). The solution was chilled overnight, and the crude product was isolated by filtration and dried. After one recrystallization from methanol followed by a second recrystallization from methanol containing glacial acetic acid, the yield of pure dye was 1.2 g. (23%), M.P. 313.5-314.5° C. dec.

25  
Dye 20.—Bis-(1,2-diphenyl-4-pyrazolidine-3,5-dione) trimethineoxonol triethylammonium salt



30  
40  
45  
1,2-diphenyl-3,5-pyrazolidinedione (1 mol., 5.05 g.), trimethoxypropene (1 mol., 1.35 g.), and triethylamine (1 mol., 2.0 g.) were dissolved in ethanol (25 ml.), and the solution was heated under reflux for fifteen minutes. The reaction mixture was chilled overnight, and the crude product was isolated by filtration and dried. After two recrystallizations from methanol, the yield of pure dye was 0.9 g. (14%), M.P. 233.5-235.0° C. dec.

50  
55  
Dye 21.—Bis-(1,2-diphenyl-4-pyrazolidine-3,5-dione) pentamethineoxonol



60  
65  
70  
75  
1,2-diphenyl-3,5-pyrazolidinedione (1 mol., 5.05 g.), 1-anilino-5-phenylimino-1,3-pentadiene hydrochloride (1 mol., 3.1 g.), and triethylamine (1 mol., 3.0 g.) were dissolved in ethanol (25 ml.), and the solution was heated under reflux for fifteen minutes. The reaction mixture was chilled overnight and then diluted with glacial acetic acid (5 ml.). The solution was chilled for several additional hours during which time ether (400 ml.) was added. The crude product was isolated by filtration and boiled with methanol (50 ml.). The mixture was cooled and diluted with glacial acetic acid (1 ml.). After chilling overnight, the crude dye was isolated by filtration and dried. After one recrystallization from methanol followed by a second recrystallization from methanol containing acetic acid, the yield of pure dye was 1.15 g. (20%), M.P. 206.5-208.5° C. dec.

Dye 22.—4-(5-acetanilido-2,4-pentadienylidene)-1,2-diphenyl-3,5-pyrazolidinedione



1,2-diphenyl-3,5-pyrazolidinedione (1 mol., 10.1 g.) and 1-anilino-5-phenylamino-1,3-pentadiene hydrochloride (1 mol., 11.4 g.) were dissolved in acetic anhydride (50 ml.), and the solution was heated under reflux for five minutes. The reaction mixture was chilled overnight, and the crude product was isolated by filtration, washed with ether, and dried. The crude dye weighed 11.8 g. (65%) and was employed without further purification as an intermediate in the preparation of additional dyes. Two recrystallizations of a sample of the crude dye (2.0 g.) from glacial acetic acid containing acetic anhydride gave 1.5 g. (75% recovery), M.P. 241.0–242.0° C.

The 1,2-disubstituted-3,5-pyrazolidinediones were prepared by conventional methods well known in the art. For example, the synthesis described by José R. Mester in Spanish Patent 212,764, issued Jan. 4, 1954, has been used advantageously. This method is abstracted in C.A., vol. 50, 8743 (1956).

In the preparation of photographic emulsions, the new dyes of the invention are advantageously incorporated in the finished silver halide emulsion and should, of course, be uniformly distributed throughout the emulsion. The methods of incorporating dyes in emulsions are relatively simple and well known to those skilled in the art of emulsion making. For example, it is convenient to add the dyes from solutions in appropriate solvents, in which the solvent selected should have no deleterious effect on the ultimate light-sensitive materials. Methanol, isopropanol, pyridine, etc. alone or in combination have proven satisfactory as solvents for the majority of our new dyes. The type of silver halide emulsions that are sensitized with our dyes include any of those prepared with hydrophilic colloids that are known to be satisfactory for dispersing light-sensitive silver halides, for example, emulsions prepared with hydrophilic colloids, such as natural materials, e.g., gelatin, albumin, agar-agar, gum arabic, alginic acid, etc., and synthetic hydrophilic resins, e.g., polyvinyl alcohol, polyvinyl pyrrolidone, cellulose ethers, partially hydrolyzed cellulose acetate, etc.

The concentration of our new dyes in the emulsion can vary widely, i.e., from about 5 to about 100 mgs. per liter of flowable emulsion. The specific concentration will vary according to the type of light-sensitive material in the emulsion and according to the effects desired. The most advantageous dye concentration for any given emulsion can be readily determined by making the tests and observations customarily used in the art of emulsion making.

To prepare a gelatino-silver halide emulsion sensitized with one of our new dyes, the following procedure is satisfactory: A quantity of the dye is dissolved in a suitable solvent, and a volume of this solution containing from 5 to 100 mgs. of dye is slowly added with intimate mixing to about 1000 cc. of a gelatino-silver halide emulsion. With most of our dyes, 10 to 20 mgs. of dye per liter of emulsion suffices to produce the maximum sensitizing effect with the ordinary gelatino-silver bromide (including bromoiodide and chlorobromide) emulsions. With fine-grain emulsions which include most of the ordinarily employed gelatino-silver chloride emulsions,

somewhat larger concentrations of dye may be necessary to secure the optimum sensitization. While the preceding has dealt with emulsions comprising gelatin, it will be understood that these remarks apply generally to any emulsions in which a part or all of the gelatin is substituted by another suitable hydrophilic colloid such as previously mentioned.

The above statements are only illustrative and are not to be understood as limiting our invention in any sense, as it will be apparent that our dyes can be incorporated by other methods in many of the emulsions customarily used in the art. For instance, the dyes can be incorporated by bathing a plate or film bearing an emulsion, in a solution of the dye.

- 15 Photographic silver halide emulsions, such as those listed above, containing the sensitizing dyes of our invention can also contain such addenda as chemical sensitizers, e.g., sulfur sensitizers (e.g., allyl thiocarbamide, thiocurea, allylisothiocyanate, cystine, etc.), various gold compounds (e.g., potassium chloroaurate, auric trichloride, etc.) (see U.S. patents to W. D. Baldsiefen, 2,540,085, granted Feb. 6, 1951; R. E. Damschroder, 2,597,856, granted May 27, 1952; and H. C. Yutzy et al., 2,597,915, granted May 27, 1952), various palladium compounds, such as palladium chloride (W. D. Baldsiefen, U.S. 2,540,086, granted Feb. 6, 1951), potassium chloropalladate (R. E. Stauffer et al., U.S. 2,598,079, granted May 27, 1952), etc., or mixture of such sensitizers; anti-foggers, such as ammonium chloroplatinate (A. P. H. Trivelli et al., U.S. 2,566,245, granted Aug. 28, 1951), ammonium chloroplatinite (A. P. H. Trivelli et al., U.S. 2,566,263, granted Aug. 28, 1951), benzotriazole, nitrobenzimidazole, 5-nitroindazole, benzidine, mercaptans, etc. (see Mees, *The Theory of the Photographic Process*, Macmillan Pub., 1942, p. 460), or mixtures thereof; hardeners, such as formaldehyde (A. Miller, U.S. 1,763,533, granted June 10, 1930), chrome alum. (U.S. 1,763,533), glyoxal (J. Brunkin, U.S. 1,870,354, granted Aug. 9, 1932), dibromacrolein (O. Block et al., Great Britain 406,750, accepted Mar. 8, 1934), etc.; color couplers, such as those described in I. F. Salminen et al., U.S. Patent 2,423,730, granted July 7, 1947; Spence and Carroll, U.S. Patent 2,640,776, issued June 2, 1953, etc.; or mixtures of such addenda. Dispersing agents for color couplers, such as those set forth in U.S. patents to E. E. Jolley et al., 2,322,027, granted June 15, 1943, and L. D. Mannes et al., 2,304,940, granted Dec. 15, 1942, can also be employed in the above-described emulsions.

Our emulsions are coated to advantage on any of the materials used for photographic elements including, for example, paper, glass, cellulose acetate, cellulose nitrate, synthetic film-forming resins, etc.

The following example will serve to further illustrate our invention by showing the sensitizing effects of representative dyes of our invention on silver halide emulsions.

#### Example 1

The representative dyes of our invention were each added, in sensitizing amounts ranging from about 20 mg. to about 170 mg. per mole of silver halide, to individual portions of a gelatino-silver bromoiodide emulsion containing 0.77 mole percent of silver iodide or a silver chlorobromide emulsion containing 40 mole percent of silver bromide (both of which are described by Trivelli and Smith, *Photographic Science*, vol. 79, 330 (1939)). After digesting for 10 minutes at 50° C., the emulsions were coated on a cellulose acetate support and dried. A sample of each coating was exposed on an IB sensitometer and to a wedge spectrogram. The exposed coatings were photographically developed for three minutes in a conventional developer solution, fixed with a conventional fixing bath, washed and dried. The sensitizing ranges and sensitizing maxima determined from the processed images are recorded with the dye and type of emulsion.

| Dye No. | Silver Halide in Emulsion | Sensitizing Range in $\text{m}\mu$ | Sensitizing Maximum in $\text{m}\mu$ |
|---------|---------------------------|------------------------------------|--------------------------------------|
| 5.....  | Silver Chlorobromide..... | To 545                             | 500                                  |
| 7.....  | Silver Bromoiodide.....   | To 550                             | 525                                  |
| 8.....  | do                        | To 550                             | 530                                  |
| 9.....  | Silver Chlorobromide..... | To 540                             | 520                                  |
| 10..... | do                        | To 600                             | 560                                  |
| 11..... | Silver Bromoiodide.....   | To 640                             | 565                                  |
| 12..... | Silver Chlorobromide..... | 510 to 640                         | 605                                  |
| 13..... | do                        | 570 to 700                         | 670                                  |
| 14..... | do                        | 660 to 735                         | 710                                  |
| 15..... | Silver Bromoiodide.....   | To 670                             | 590                                  |
| 21..... | Silver Chlorobromide..... | 580 to 650                         | 620                                  |
| 22..... | do                        | 490 to 550                         | 525                                  |

Certain of our dyes, for example, dyes 11, 13, 17, 18, 19, 20 and 21 are bleached by photographic developer solutions and are therefore useful as dyes for light-filtering layers in photographic elements.

Certain dyes of our invention derived from 1,2-disubstituted-3,5-pyrazolidinediones are valuable spectral sensitizers for photographic silver halide emulsions and photographic elements coated therefrom. The preferred sensitizers include the merocyanines, holopolar dyes, and oxonols. Other dyes of our invention are bleachable by photographic developers and find use as filter dyes in photographic elements.

The invention has been described in considerable detail with particular reference to certain preferred embodiments thereof, but it will be understood that variations and modifications can be effected within the spirit and scope of the invention as described hereinabove and as defined in the appended claims.

We claim:

1. A dye selected from those having the formulas:



and



wherein R and R' each represent a group selected from the class consisting of an alkyl group and an aryl group; R<sup>2</sup> represents a group selected from the class consisting of an alkyl group and an aryl group; L and L' each represent a methine group; r represents an integer of from 1 to 3; and W and W' each represent the nonmetallic atoms required to complete a 5 to 6 membered heterocyclic nucleus selected from nuclei of the class consisting of nuclei of the thiazole series, nuclei of the benzothiazole series, nuclei of the naphthothiazole series, nuclei of the thionaphtheno-7',6',4,5-thiazole series, nuclei of the oxazole series, nuclei of the benzoxazole series, nuclei of the naphthoxazole series, nuclei of the selenazole series, nuclei of the benzoselenazole series, nuclei of the naphthoselenazole series, nuclei of the thiazoline series, nuclei of the 2-quinoline series, nuclei of the 4-quinoline series, nuclei of the 1-isoquinoline series, nuclei of the 3-isoquinoline series, nuclei of the 3,3-dialkylindolene series, nuclei of the pyridine series, and q represents an integer of 1-2; R<sup>3</sup>

and  $R^4$  represent alkyl groups and  $m$  represents an integer from 1 to 2.

2. A dye of claim 1 having Formula I.
  3. A dye of claim 1 having Formula II.
  4. The dye bis-(1,2-diphenyl-4-pyrazolidine-3,5-dione) pentamethineoxonol.
  5. A light-sensitive photographic emulsion comprising a hydrophilic colloid, silver halide and a dye selected from those having the formulas:



35 wherein R and R' each represents a group selected from the class consisting of an alkyl group and an aryl group; R<sup>2</sup> represents a group selected from the class consisting of an alkyl group and an aryl group; L and L' each represent a methine group; r represents an integer of from 1 to 3; and W and W' each represent the nonmetallic atoms 40 required to complete a 5 to 6 membered heterocyclic nucleus selected from nuclei of the class consisting of nuclei of the thiazole series, nuclei of the benzothiazole series, nuclei of the naphthothiazole series, nuclei of the thionaphtheno-7',6',4,5-thiazole series, nuclei of the oxazole 45 series, nuclei of the benzoxazole series, nuclei of the naphthoxazole series, nuclei of the selenazole series, nuclei of the benzoselenazole series, nuclei of the naphthoselenazole series, nuclei of the thiazoline series, nuclei of the 2-quinoline series, nuclei of the 4-quinoline series, nuclei 50 of the 1-isoquinoline series, nuclei of the 3-isoquinoline series, nuclei of the 3,3-dialkyldolene series, nuclei of the pyridine series, and q represents an integer of 1-2; R<sup>3</sup> and R<sup>4</sup> represent alkyl groups and m represents an integer from 1 to 2.

- 55 6. A photographic element comprising a support, at least one hydrophilic colloid layer containing light-sensitive silver halide and at least one hydrophilic colloid layer containing a dye selected from those having the formulas:



and

(III)



wherein R and R' each represents a group selected from the class consisting of an alkyl group and an aryl group; R<sup>2</sup> represents a group selected from the class consisting of an alkyl group and an aryl group; L and L' each represent a methine group; r represents an integer of from 1 to 3; and W and W' each represent the nonmetallic atoms required to complete a 5 and 6 membered heterocyclic nucleus selected from nuclei of the class consisting of nuclei of the thiazole series, nuclei of the benzothiazole series, nuclei of the naphthothiazole series, nuclei of the thionaphtho-7',6',4,5-thiazole series, nuclei of the oxazole series, nuclei of the benzoxazole series, nuclei of the naphthoxazole series, nuclei of the selenazole series, nuclei of the benzoselenazole series, nuclei of the naphthoselenazole series, nuclei of the thiazoline series, nuclei of the 2-quinoline series, nuclei of the 4-quinoline series, nuclei of the 1-isoquinoline series, nuclei of the 3-isoquinoline series, nuclei of the 3,3-dialkylindolene series, nuclei of the pyridine series, and q represents integer of

1-2; R<sup>3</sup> and R<sup>4</sup> represent alkyl groups and m represents an integer from 1 to 2.

7. A light-sensitive photographic emulsion comprising a hydrophilic colloid, silver halide, and the dye bis-(1,2-diphenyl - 4 - pyrazolidine-3,5-dione)pentamethine-oxonol.

## References Cited

## UNITED STATES PATENTS

|           |         |                  |           |
|-----------|---------|------------------|-----------|
| 2,272,163 | 2/1942  | Kendall          | 96-102    |
| 2,427,911 | 9/1947  | Kendall et al.   | 260-310   |
| 2,639,282 | 5/1953  | Sprague et al.   | 96-102    |
| 2,895,955 | 7/1959  | Haseltine et al. | 260-240.5 |
| 2,984,664 | 5/1961  | Fry et al.       | 260-240.5 |
| 2,955,939 | 10/1960 | Brooker et al.   | 96-105    |
| 2,965,486 | 12/1960 | Brooker et al.   | 96-105    |

## FOREIGN PATENTS

|         |        |                |
|---------|--------|----------------|
| 781,551 | 8/1957 | Great Britain. |
|---------|--------|----------------|

## OTHER REFERENCES

Cardani et al., Faemaco, Ed. Sci. vol. XI, pp. 336-345 (1956).

Zenno, Chemical Abstracts, vol. 48, pp. 11063-4 (1954).

J. TRAVIS BROWN, Primary Examiner.

NORMAN G. TORCHIN, Examiner.